

Dec. 3, 1968

E. ZUR

3,413,798

YARNS AND FABRICS THEREOF

Filed March 6, 1967

**F I G. 1**



**F I G. 1A**



**F I G. 2**



**F I G. 2A**



INVENTOR

EITAN ZUR

BY

*Eugene Berman*

AGENT

1

3,413,798

**YARNS AND FABRICS THEREOF**

Eitan Zur, Wilmington, Del., assignor to E. I. du Pont de Nemours and Company, Wilmington, Del., a corporation of Delaware

Filed Mar. 6, 1967, Ser. No. 621,049  
12 Claims. (Cl. 57—140)

**ABSTRACT OF THE DISCLOSURE**

A composite yarn composed of an inelastic continuous filament yarn combined with staple fibers having specific work-to-break and tenacity values, the continuous filament yarn being visible among the staple fibers in the composite yarn. A knit fabric of these yarns having unique aesthetics, namely, a silk-life appearance and a tactility combining worsted-like and silk-like hand.

This invention relates to novel yarns. The invention also relates to novel, pill-free, knitted fabrics, which have a silk-like appearance and a highly unusual tactility combining worsted-like and silk-like hand, which are formed from these novel yarns.

A problem encountered in producing fabrics from staple yarns, both natural and synthetic, is that the staple fibers in the resulting fabrics have a tendency during use to associate together in the form of small balls or "pills" which give the fabric an unsightly appearance. Pilling is especially severe in knitted staple fabrics, since the yarns used in knitted fabrics usually have less twist than the yarns used in woven fabrics and fabric construction is generally looser. Synthetic fibers of both the acrylic and polyester type are now available in which the toughness of the fibers has been deliberately minimized so that pills, when formed, will break off rather readily. Although the number of pills found on fabrics made from such fibers is lower than the level previously considered normal, some pills are usually seen at any given time after the fabric has been placed in use. Accordingly, a continuing need has been felt for the development of fabrics upon which pills are seldom seen, if ever, and which accordingly could be described as "pill-free."

It is an object of this invention to provide novel yarns. Another object is to provide pill-free knitted fabrics from these novel yarns.

*Statement of the invention*

In accordance with this invention, a composite yarn is provided composed of inelastic continuous filament yarn combined with staple fibers having a work-to-break of less than about 0.5 gm. cm./denier cm., at least 30 wt. percent of said staple fibers being acrylonitrile polymer staple fibers having a tenacity of less than 1.5 g.p.d., the continuous filament yarn being visible among the staple fibers in the composite yarn.

The novel fabric of the invention is a knit fabric of the composite yarn defined above.

*Description of the preferred embodiments of the invention*

In one preferred embodiment of the invention, the yarn is a core-spun yarn in which the staple fibers form a sheath around the continuous filament core, with the continuous filament being off-center and close enough to the side of the yarn that it is visible among the staple fibers in the composite yarn. The knit fabric produced from this yarn has a subtle, highly attractive differential luster. Its hand, although somewhat silk-like also has a worsted-like tactile impression, all the more surprising because of the silk-like appearance of the fabric.

2

In another preferred embodiment of the invention, the staple fibers are twisted in the form of a staple yarn which in turn is ply-twisted about the continuous filament yarn. In this embodiment of the invention, the continuous filament is even more readily apparent than in the core-spun yarn. The knit fabric produced from this yarn has a high degree of differential luster. Its hand also has a marked worsted-like tactile impression, although the tactility of this fabric is more silk-like than that of the fabric made from the core-spun yarn of the invention.

In a particularly preferred embodiment of the invention, the staple fibers in the composite yarn are a blend in which from 30% to 70% of the fibers are acrylonitrile polymer fibers and the remaining 70% to 30% are polyester fibers.

The knit fabric formed from the novel yarns of the invention may be of any knit construction, but the preferred fabrics are double knit fabrics, since the silk-like differential luster and luxurious tactility reach their optimum in fabrics of double-knit construction.

Yarn according to this invention is illustrated in the attached drawing in which:

FIGURE 1 illustrates a side view of a core-spun composite yarn;

FIGURE 1A is a cross-sectional view of the core-spun composite yarn of FIGURE 1;

FIGURE 2 illustrates a side view of a plied composite yarn; and

FIGURE 2A is a cross-sectional view of the plied composite yarn of FIGURE 2.

*Definition of terms*

The term "composite yarn" as used herein, and generally in the art, refers to yarn composed of two or more yarns combined together by core-spinning, plying, wrapping or equivalent methods of combining yarn. "Core-spinning" refers to the process of introducing continuous filament to a conventional spinning or drafting frame together with one or more rovings of staple fibers to produce a composite yarn having the continuous filament as a core and the drafted rovings as a sheath (note, for example, U.S. Patent 3,017,740 to Humphreys). "Plying" refers to a method wherein two or more yarns are plied (i.e., twisted together) to form a composite yarn. (Note, for example, U.S. Patent 2,656,585 to Jackson.) "Wrapping" refers to a method wherein continuous filament yarn is wrapped with one or more layers of staple fiber yarn. (Note, for example, U.S. Patent 2,024,156 to Foster.) The term "composite yarn" is to be distinguished from the term "composite fiber." One or more of the fiber components of the "composite yarn" may suitably be "multicomponent fiber," the latter term refers to a fiber containing two or more fiber-forming components in an eccentric relationship over the cross section of the fiber and throughout the length of the fiber. (Note, for example, U.S. Patent 3,039,524.)

The term "work-to-break" as used herein, and generally in the art, is a measure of the amount of work (e.g., gram-centimeter) necessary to break a fiber and is given in units of gram-centimeters/denier centimeter. This term gives tensile strength properties in addition to those specified by "tenacity" which is a measure of the breaking strength of the fiber, i.e., the force (e.g., grams) necessary to break the fiber.

The term "inelastic" used in reference to continuous filament yarn refers to any conventional, tenacious, textile yarn prepared from a synthetic polymer, such as polyesters, acrylonitrile polymers, polyamides, e.g., nylon 6,6, polyolefins, e.g., polypropylene, which require a considerable force (e.g., greater than about 0.15 g.p.d.) to elongate to a low elongation (e.g., less than about 1%) with permanent deformation occurring at a relatively low

elongation (e.g., 5% or less). Although all yarns have some measurable elasticity, the term serves to distinguish conventional textile continuous filament yarns from conventional elastic yarns which require little force to elongate them markedly and which subsequently retract to their initial length when the force is released.

The term "continuous filament yarn" as used herein includes both monofilament and multifilament continuous yarns. A wide range of denier is suitable. A total yarn denier of from about 30 to about 60 is preferred (about 40 denier being most preferred) for most end uses.

The term "staple fiber," as used herein, refers to continuous filaments cut or broken into relatively short fiber lengths. The length of these fibers is chosen by reference to the particular spinning system used to prepare yarn from these fibers (e.g., if yarn is to be spun on the woolen system, the fiber is cut to the staple length of natural wool). A wide range of denier is suitable. A staple fiber denier of from about 2 to about 4.5 is preferred (about 3 denier being most preferred for most end uses).

The term "acrylonitrile polymer" as used herein, includes any long chain synthetic polymer composed of at least 35 (preferably at least 85) percent by weight of acrylonitrile units of the formula



in the polymer chain. As is well understood, the term includes the homopolymer of acrylonitrile and polymers of acrylonitrile and monoethylenically unsaturated monomers polymerizable with acrylonitrile. Nonlimitative examples of preferred comonomers include styrene, 2-vinylpyridine, 2-methyl-5-vinylpyridine, 4-vinylpyridine, methyl acrylate, sodium styrene sulfonates, vinylidene chloride, and vinyl acetate.

The term "polyester" refers to a polycondensation polymer with recurring units of the formula



constituting an integral part of the polymer chain. The polyester is preferably a polymer of a glycol and a dicarboxylic acid in which the repeating structural units of the polyester contain at least one aromatic nucleus having chain-extending valence bonds separated by a minimum of four nuclear carbon atoms. Nonlimitative examples of preferred polyesters include polyethylene terephthalate alone or as a copolymer with ethylene 5-sodium sulfo) isophthalate or ethylene hexahydroterephthalate.

To achieve the objectives of this invention the staple fibers twisted about the continuous filament yarn should have a work-to-break of less than about 0.5 gm. cm./denier cm. Staple fibers of low toughness are required in the yarns of this invention in order that aggregations of fuzzed staple fibers approaching the dimensions of a pill will be sheared off. It is believed that this occurs as the result of the continuous filament yarn acting as a dull knife blade, although this statement is not intended as limiting. At least 30% of the staple fibers in the composite yarn should be acrylonitrile polymer fibers having a tenacity of less than about 1.5 grams per denier (g.p.d.). When a pill begins to form from fuzzed staple fibers in a garment, these low-toughness, low-tenacity acrylonitrile polymer fibers break readily and thereby contribute markedly to the elimination of the pill while it is still small or incipient, by the self-action of the novel yarn. The characteristic desirable aesthetics of acrylonitrile polymer staple fibers are imparted to the fabric by the presence of these fibers to the extent of at least 30% among the staple fibers. Preferably, acrylonitrile polymer bicomponent staple fibers having a work-to-break of less than about 0.5 gm. cm./denier cm. and a tenacity of less than

1.5 g.p.d. are used. These bicomponent fibers impart increased bulk to the fabric, which enhances the luxurious tactility of the fabric.

If desired, all of the staple fibers may be acrylonitrile polymer staple fibers; however, up to 70% of the staple fibers may be polyester staple fibers or other staple fibers so long as their work-to-break does not exceed 0.5 gm. cm./denier cm. The tenacity of these fibers may be higher than the tenacity of the acrylonitrile polymer fibers, and if so the acrylonitrile polymer fibers may break first in incipient pills to weaken their attachment to the fabric, but the low toughness of any remaining fibers leads to early elimination of pills by the self-action of the novel yarn.

It is important that the continuous filament yarn be visible (i.e., that it show through and be visible to the unaided human eye among the staple fibers) in the composite yarn; so that the continuous filament yarn is not completely "covered." This is believed to be an important factor in the silk-like appearance, as well as the improved pill resistance, of the knit fabric. The methods for preparing "composite" yarn (previously mentioned) must be practiced under conditions which provide this incomplete "cover." In "plying," the twisting together of the yarns generally results in the continuous filament being visible. In "core-spinning" a small displacement of the continuous filament yarn from the edge of the staple fiber roving as it is fed into the spinning frame will generally result in the incomplete cover. In "wrapping," it is necessary to incompletely wrap the continuous filament yarn with staple fiber yarn (i.e., allow intermittent portions of the continuous filament yarn to be left uncovered).

Composite yarn having these characteristics is illustrated in the drawing:

35 In FIGURE 1, a core-spun composite yarn 10 is illustrated. The continuous filament yarn 12 is the core with a sheath of staple fibers 14. The continuous filament yarn 12 is off-center and closer to the side of the composite yarn 10, and is visible among the staple fibers 14.

40 In FIGURE 2, a plied composite yarn 20 is illustrated. The continuous filament yarn 22 is twisted together with the staple fibers 24 in a ply formation, i.e., neither is wrapped as a cover about the other as a core but rather both follow generally similar paths about each other. The continuous filament yarn 22 is visible among the staple fibers 24 in the composite yarn 20.

45 The relative weights of continuous filament yarn and staple fiber may be varied in the composite yarn to provide different degrees of "cover," resulting in variations in the tactility and luster of the knit fabric end product. Increasing amounts of continuous filament yarn generally results in a more silk-like tactility as well as a more silk-like luster. Decreasing amounts in turn result in these properties being more worsted-like. The continuous filament yarn must be present to provide improved pill resistance. For most purposes to achieve a unique balance of silk-like and worsted-like properties from about 10 to about 40 weight percent of continuous filament yarn is preferred. A most preferred range is from about 10 to about 30 weight percent. As is evident from the above discussion, one skilled in the art may vary these percentages for various end use requirements.

#### EXAMPLES

55 The preferred embodiments of the invention will be illustrated by the examples that follow. Parts and percentages are by weight unless otherwise indicated.

#### EXAMPLE I

70 This example illustrates a preferred core-spun yarn and knit fabric according to this invention.

A roving comprising a blend of equal weights of staple fibers is prepared from the following starting materials:

*Fiber A.*—A bicomponent acrylic fiber in which the components are a mixture of polymers, the first of which

has a composition of 95.25 wt. percent acrylonitrile, 3.25 wt. percent sodium styrenesulfonate and 1.50 wt. percent methyl acrylate, and the second component has a composition of 99.29% acrylonitrile, 0.22 wt. percent methyl acrylate, and 0.49 wt. percent of sodium styrenesulfonate.

The fibers have a denier per filament of 3.5, a tenacity of 0.94 g.p.d., an elongation of 43.7%, a toughness (work-to-break) of 0.39 gm. cm./denier cm., and are in the form of a tow of about 470,000 denier.

*Fiber B.*—A polyester fiber of polyethylene terephthalate/5-(sodium sulfo)isophthalate (98/2) having a relative viscosity of about 12. The fibers have a denier per filament of 3.0, a tenacity of 2.2 g.p.d., an elongation of 25%, a toughness of 0.35 gm. cm./denier cm., and are in the form of a tow having a denier of about 470,000.

The roving is prepared by feeding two ends each of the Fiber A and Fiber B tows to a Pacific Converter and cutting them to a vari-cut length of 4.5 inches (11.4 cm.) to form a sliver, which is then blended by pin-drafting and formed into a one-hank roving on a conventional worsted system.

The roving so prepared is core-spun with a continuous filament yarn designated as "Fiber C" and more fully identified as follows:

*Fiber C.*—A bright, 40-denier continuous filament polyethylene terephthalate yarn having a relative viscosity of about 28 and comprised of 8 filaments. In contrast to the low toughness of the polyester fiber designated above as Fiber B, typical values for this polyester fiber are a work-to-break of 0.75 gm. cm./denier cm., a tenacity of 4.6 g.p.d., and an elongation of 30%.

In preparing the core-spun yarn, the roving is given a draft of 17.77 on a spinning frame set to give a 1/40 worsted count yarn having a 15 Z twist, and the filament yarn ("Fiber C") is fed about 0.125 inch (0.318 cm.) to the left of the left edge of the roving at the delivery roll. The product is a 1/33.3 worsted count yarn having a denier of 239 and composed of 42% by weight of the acrylic sheath fibers ("Fiber A"), 42% of the polyester sheath fibers ("Fiber B"), and 16% by weight of the continuous filament polyester yarn ("Fiber C"). The presence of the continuous filament yarn in the resulting core-spun yarn is readily apparent, since it is only partially hidden by the staple fibers in the sheath. The yarn has a Lea Product of 2165 and a Coefficient of Variance of 15.0%.

The sheath-core yarn so prepared is knit on an 18-cut Dubied "Wevenit" circular weft knitting machine using a Swiss Double Pique stitch. The knitted greige fabric has a weight of 9.6 ozs./sq. yd. (325 grams/sq. meter) after steaming. Excellent knitting performance is observed.

The knitted fabric is heat-set on a frame in 350° F. air under tension for an exposure time of 2 minutes. The fabric is then scoured and dyed according to the following procedure, in which all percentages are based on fabric weight. The scouring is carried out in an aqueous 1.0% solution of nonionic detergent for 15 minutes at 160° F. (71° C.). The dye solution, at a 40:1 bath to fiber ratio, comprises 0.03% sodium acetate, 0.5% of the non-ionic detergent, 20.0% sodium sulfate, and 1.5% of C.I. (Colour Index) Basic Red 22 dye. The dyebath is adjusted to a pH of 4.5 with acetic acid, the temperature is raised to 212° F. (100° C.), and the fabric is dyed for 30 minutes. The dyebath is then cooled and 0.46% of C.I. Disperse Yellow 54 dye, 0.01% of C.I. Disperse Blue 61 dye, and 2.5 grams/liter of dispersed butyl benzoate are added. The pH is adjusted to 7.0 with tetrasodium pyrophosphate, the bath is again heated to 212° F. (100° C.), and dyeing is carried out for an additional hour. The fabric is then removed from the dyebath, rinsed, tumble dried at 180° F. (82° C.), steam calendered about 5% over the as-dried width, and semi-decated with a 1-minute exposure to steam and a 1-minute exposure to vacuum.

The dyed and finished fabric has a luxurious differential luster, quite unlike knitted fabrics of conventional staple

blend yarns. The fabric has unusual, highly luxurious aesthetics characterized by a high degree of liveliness, excellent drape, and tactility combining worsted-like and silk-like hand. The fabric performance in wear is outstanding and is characterized by no detectable pilling, after 200 hours of wear, in a dress made of the fabric. When the dress is worn 200 hours with five total dry cleanings (every 40-50 hours), the fabric appears virtually unchanged with respect to the fabric in a similar dress of the same material which has never been worn.

The pilling propensity of the dyed and finished fabric is evaluated on the "Random Tumble Pilling Tester" described by E. M. Baird, L. C. Legere, and H. E. Stanley in Textile Research Journal, vol. 26, pages 731-735 (1956). The following scale of pill level ratings is employed in evaluating fabrics in this test:

- 5.0—no pilling
- 4.0—slight pilling
- 3.0—moderate pilling
- 2.0—heavy pilling
- 1.0—severe pilling

Intermediate ratings within the above values are assigned to the nearest 0.1 unit to place fabrics in their proper rank in the above scale. Three samples of each fabric are rated, and the ratings are averaged.

The dyed and finished fabric of the example, designated as the "Test Fabric," is compared with a "Control Fabric" double knit from a yarn composed of staple fibers only, prepared from a blend of equal weights of Fiber A and Fiber B. The weight, construction, dyeing, and finishing of the "Control Fabric" are similar to those of the "Test Fabric." The results are as follows:

|                       | Random tumble pill test rating |        |         |
|-----------------------|--------------------------------|--------|---------|
|                       | 3 min.                         | 5 min. | 10 min. |
| "Test Fabric"-----    | 5.0                            | 5.0    | 5.0     |
| "Control Fabric"----- | 4.4                            | 4.3    | 4.5     |

Actual performance during wear correlates with laboratory results in garments made from the above fabrics, the "Control Fabric" garment being rated an average of 0.5 unit lower than the "Test Fabric" garment after wear periods of 100, 150, and 200 hours.

The above pilling data clearly indicates that although the staple fiber properties (e.g., work-to-break, tenacity) are important in providing relatively good pill resistance, the continuous filament yarn, as also required by the present invention, is necessary to achieve the high degree of pill resistance desired.

## EXAMPLE II

This example illustrates a preferred plied yarn and knit fabric according to this invention.

A quantity of the roving of Example I is spun into a 1/40 worsted count staple yarn having a 15 Z twist, a Lea Product of 1560, and a Coefficient of Variance of 17.7%. The completed staple yarn is ply twisted at the twister together with the continuous filament polyester yarn designated as "Fiber C" of Example I. The yarn is plied to achieve a balanced twist, requiring approximately 4 S twist. The plied yarn so produced is a 239 denier, 1/33.3 worsted count yarn having a Lea Product of 2340 and a Coefficient of Variance of 16.7%. The presence of the continuous filament yarn in the plied yarn is readily apparent.

A double-knit fabric is prepared from the plied yarn, following the procedure of Example I, except that the knitted greige fabric has a weight of 8.3 ozs./sq. yd. (281 grams/sq. meter) after steaming. The knitted fabric is heat-set, dyed, and finished in the same way as the knitted fabric of Example I, except that in the dyeing step the following basic dyes are substituted in place of the basic dye employed in Example I: 3.34% C.I. Basic Blue 35 dye, 3.34% C.I. Basic Blue 21 dye, 0.786% C.I. Basic

Yellow 15 dye, 0.607% C.I. Basic Red 18 dye; while 0.46% C.I. Disperse Yellow 54 dye is again used and the amount of C.I. Disperse Blue 61 dye is increased to 2.53%.

The knitted fabric so prepared and finished has a high degree of differential luster, more pronounced than the luster of the fabric of Example I. The fabric is very lively and has excellent drape, being in this respect very similar to the fabric of Example I. The tactility of the fabric combines both worsted-like and silk-like hand; with respect to the fabric of Example I, it is somewhat more silk-like. The fabric performance in wear is outstanding and is characterized by no detectable pilling, after 200 hours of wear, in a dress made of the fabric. When the dress has been worn 200 hours with five total dry cleanings (every 40-50 hours), little difference is observable between the dress which has been worn and a similar dress which has never been worn.

The knitted fabric, after finishing, is given ratings of 5.0 on the "Random Tumble Pilling Tester" after test periods of 3, 5 and 10 minutes, correlating with actual wear performance similar to that of the "Test Fabric" of Example I and up to 0.5 unit higher than the "Control Fabric" ratings during actual wear. These results further confirm the additional importance of the required continuous filament yarn.

As the examples illustrate, the performance in wear of the knit fabric is outstanding, and is characterized by no detectable pilling after 200 hours of wear in garment form. Garments of the fabric, worn for 200 hours with five total dry cleanings (every 40-50 hours), are remarkably fresh looking and difficult to distinguish from unworn garments. The significant effect of the presence of continuous filament yarn on pilling is clearly shown. Most surprising, however, is the unexpected appearance of the fabrics with their silk-like differential luster; their excellent drape and liveliness; and especially their unusual tactility, or hand. The hand of the fabrics is characterized by a marked worsted-like tactile impression, very unlike that of conventional knitted fabrics. The hand is perhaps best described as intermediate between silk-like and worsted-like.

The great and varied utility for these novel yarns and fabrics will be obvious to those skilled in the art.

The foregoing specification is intended to be descriptive of the invention, but due to the possible variations it is not in limitation thereof. The scope of the invention is defined by the following claims.

What is claimed is:

1. Composite yarn comprising inelastic continuous filament yarn combined with staple fibers, said staple fibers having a work-to-break of less than about 0.5 gram-centimeter/denier-centimeter, at least about 30 weight percent of said staple fibers being acrylonitrile polymer staple fibers having a tenacity of less than about 1.5 grams per denier, the said continuous filament yarn being visible among said staple fibers in said composite yarn.
- 10 2. Core-spun composite yarn according to claim 1.
3. Plied composite yarn according to claim 1.
4. Composite yarn according to claim 1 wherein said continuous filament yarn comprises from about 10 to about 40 weight percent of said composite yarn.
- 15 5. Composite yarn according to claim 4 wherein said continuous filament yarn weight percent is less than about 30.
- 20 6. Composite yarn according to claim 1 wherein said continuous filament yarn has a total yarn denier of from about 30 to about 60 and said staple fiber has a fiber denier of from about 2 to about 4.5.
- 25 7. Composite yarn according to claim 1 wherein said staple fibers are a blend in which from about 30 to 70 weight percent are acrylonitrile polymer fibers and 70 to 30 weight percent are polyester fibers.
8. Composite yarn according to claim 1 wherein said acrylonitrile polymer contains at least 85 weight percent of recurring acrylonitrile units.
- 30 9. Composite yarn according to claim 1 wherein said acrylonitrile polymer staple fibers are multicomponent fibers.
- 35 10. Composite yarn according to claim 1 wherein said continuous filament yarn is prepared from a synthetic polymer selected from the group consisting of polyesters, acrylonitrile polymers, polyamides and polyolefins.
11. Knit fabric containing the composite yarn of claim 1.
12. Double knit fabric containing the composite yarn of claim 1.

#### References Cited

##### UNITED STATES PATENTS

|           |        |               |       |           |
|-----------|--------|---------------|-------|-----------|
| 2,890,567 | 6/1959 | Taylor et al. | ----- | 57-140    |
| 3,038,295 | 6/1962 | Humphreys.    |       |           |
| 3,081,516 | 3/1963 | Evans         | ----- | 57-140    |
| 3,365,875 | 1/1968 | Hall          | ----- | 57-140 XR |

FRANK J. COHEN, Primary Examiner.

D. WATKINS, Assistant Examiner.